

## UNITED STATES PATENT OFFICE.

KARL MÜLLER AND WILHELM SANDEE, OF ESSEN, GERMANY.

## BEARING METAL ALLOY.

No Drawing.

Application filed August 29, 1921. Serial No. 496,632.

*To all whom it may concern:*

Be it known that we, KARL MÜLLER and WILHELM SANDER, citizens of the German Republic, and residing at Essen, Germany, 5 have invented a new and useful Improvement in Bearing Metal Alloys; and we do hereby declare the following to be a full, clear, and exact description of the same.

This invention relates to bearing metal 10 alloys with the characteristic feature of a high (75 to 80 per cent) lead content.

Bearing metals of this type have latterly been frequently and largely employed in 15 practice. Alloys of this kind have approximately the following composition: about 80 per cent of lead, about 10 to 15 per cent of antimony, about 5 to 10 per cent of tin, together with small intentional additions of copper.

20 Nevertheless up to the present the field of technical application of such bearing metals of high lead content has been limited.

In the case of heavy loads a bearing metal with high tin content had always to be used. 25 The alloys of the above composition high in lead have mostly an insufficient degree of hardness, usually below or approximately 20 Brinell. Moreover, when submitted to heavy strains and especially when the lubrication fails these bearing metals tend to crumble (or scale), individual small parts of the bearing becoming detached, a disadvantage which at once produces hot running and thus causes serious interference with the 30 working of the machine. This tendency to crumble is especially dangerous when the direction of rotation is suddenly changed, as often happens in railway shunting.

According to our invention these drawbacks are avoided and the properties of such bearing metals as mentioned above, consisting mainly of lead, and containing antimony and tin are considerably improved by a small percentage, say about 0.5 per cent of 40 phosphorus, which is added to the alloy in question. The addition of phosphorus increases the Brinell hardness by more than 50 per cent, such improved bearing metals having generally a Brinell hardness of above 45 30. At the same time however, the addition of phosphorus produces such an improvement in the physical properties of the alloy, that the tendency to crumble (scale) and

abrasion disappears. Practical experiments have shown that bearing metals high in lead, 55 which have been improved by the introduction of phosphorus, will give the same technical results as a high-grade white metal alloy containing tin. These new bearing metals may therefore be regarded as fully 60 equivalent substitutes for the latter.

The introduction of phosphorus into the alloy high in lead may be effected directly, but preferably by using an intermediate 65 alloy. As such, the alloy of phosphorus-copper; phosphorus - manganese - copper; phosphorus-zinc and phosphorus-brass have been found to be specially suitable. Apart from facilitating the introduction of the phosphorus, the above phosphorus alloys 70 have the advantage of further improving the properties of the bearing metal, increasing the Brinell hardness, and also ensuring the more reliable working of the bearings.

Furthermore, we have found that the addition of a very small amount of iron (up to about 1 per cent) considerably diminishes the brittleness of the alloy under consideration increasing at the same time its toughness.

80 What we claim is:

1. A bearing metal alloy comprising approximately eighty per cent of lead, the balance including antimony and tin in amounts not less than ten per cent and five 85 per cent respectively, and approximately 0.5 per cent of phosphorus.

2. A bearing metal alloy consisting mainly of lead, and containing about 10 to 15 per cent of antimony, about 5 to 10 per cent of 90 tin, and about 0.5 per cent of phosphorus.

3. A bearing metal alloy comprising approximately eighty per cent of lead, the balance including antimony and tin in amounts not less than ten per cent and five 95 per cent respectively, and a small percentage of phosphorus.

In testimony whereof, we have signed our names to this specification in the presence of two subscribing witnesses.

DR. KARL MÜLLER.

DR. WILHELM SANDER.

Witnesses:

AUGUST WALTER,  
FRITZ RUHL.